

Aug. 19, 1924.

1,505,401

E. MAYER

CASTING AND IN THE PROCESS FOR ITS MANUFACTURE

Filed March 14, 1922

*Fig. 1*



*Fig. 2*



Inventor:

E. Mayer

By *Lawrence K. Burgess*  
Attorney.

Patented Aug. 19, 1924.

1,505,401

# UNITED STATES PATENT OFFICE.

ERNEST MAYER, OF ANTWERP, BELGIUM.

## CASTING AND IN THE PROCESS FOR ITS MANUFACTURE.

Application filed March 14, 1922. Serial No. 543,754.

To all whom it may concern:

Be it known that I, ERNEST MAYER, a subject of the King of Belgium, and resident of Antwerp, Belgium, have invented 5 certain new and useful Improvements in Castings and in the Processes for their Manufacture; and I do hereby declare the following to be a full, clear, and exact description of the invention, such as will enable others skilled in the art to which it 10 pertains to make and use the same, reference being had to the accompanying drawings, and to letters or figures of reference marked 15 therein, which form a part of this specification.

In some castings in iron or steel it is of frequent occurrence to find defects due to porous places, unequal shrinkage and accidental blow-holes, which necessitates 20 scrapping the castings even when the latter appear good and uniform and well moulded on careful visual inspection so that it is only after being machined and being subjected to pressure tests that the castings 25 show want of tightness.

These defects are particularly serious and objectionable in the case of certain articles such as the cylinders for motor-car, aero- 30 plane engines, and locomotives, hydraulic piping and presses, etc.

The present invention has now for its object to obviate the above mentioned defects.

This object is effected by joining to the 35 mass of the castings, in pouring the metal a solid plate or sheet of metal of such shape and dimensions that the walls of the castings which are strengthened or rendered tight thereby are thus composed partly of ordinary casting metal and partly of 40 rolled or drawn sheet of metal having a higher melting point, this part of rolled sheet constituting one or more of the walls of the castings.

Owing to the temperature to which this sheet of metal is subjected during the pouring operation an intimate union takes place 45 between the two parts of the castings.

The walls of the castings thus produced 50 are rendered fluid-tight and are also strengthened owing to the pressure of this sheet of metal.

On the other hand the presence of this 55 rolled or drawn sheet of metal acts, during the pouring operation, chemically and physically upon the quality of the casting

metal that is situated in its immediate vicinity. For instance the casting metal in contact with the sheet of soft steel becomes 60 decarburized and the grain of the casting metal is thereby rendered finer so that the casting metal becomes stronger and more fluid-tight.

The sheets of metal are usually rolled and of flat, tubular, or dished form, or drawn 65 in the form of tubes, and they may be covered with a suitable metal or coating. For instance, they may be previously tinned.

The shape of these sheets of metal depends 70 necessarily on the shape of the walls of the casting. In the application of this invention to a cylindrical article (engine cylinder, press cylinder, pipe, etc.) the sheet of metal consists simply of a tube or of 75 a metal sheet bent in the form of a tube. When the invention is applied on the contrary to walls of more complicated form, such as cylinder jackets, valve chests, etc., the shape of the metal plate is usually produced 80 by dishing or profile-shaping.

It is to be noted that the process, according to the invention, which has as result the obtaining of castings having walls of mixed composition, comprising a part of 85 cast-iron and a part of metal sheet, this latter being placed on one of the faces of the walls, is essentially different to the process which consists in obtaining castings having a sheet of metal placed near the mid- 90 dle of the wall, this sheet serving to the strengthening of the casting.

The accompanying drawings illustrate by way of example the positioning of these 95 metal sheets in the case of an internal combustion engine cylinder, and in the case of a tube.

Figure 1 is a section of an internal combustion engine cylinder and other elements forming the casting.

Figure 2 is a section of a tube.

As shown in Figure 1, the arrangement is as follows:—

A tubular metal sheet 1 inserted in the cylindrical portion of the engine cylinder. 105

A dished metal sheet 2 inserted in the head.

A cylindrical metal sheet 3 arranged around the suction pipe.

A metal sheet 4 arranged around the ex- 110 haust valve chest.

A cylindrical metal sheet 5 arranged

around the socket for the sparking plug. It is to be noted that according to circumstances, according to the nature of the metal, and the quality of the castings to be produced it is optional to use plates or sheets or tubes of any suitable shape and material, these metal sheets being joined afterwards to the walls of the casting.

In the case of Figure 2, a plate 6 is provided which is placed on the outer surface of the casting tube, and another plate 7 which is arranged on the inner surface of the said tube.

It is to be noted that in the case of the pouring of castings having a complicate form as cylinder-blocks for internal combustion engines (Fig. 1) or other pieces presenting variable thicknesses, the use of metal sheets, according to the present invention, prevents the contraction of the cast iron and consequently the defects of leakage on the spots where the variation of the thickness of said pieces is notable.

In considering, by way of example, the spot 8, where the outer surface of the cooling jacket 9 is joined to the cylinder properly so called. The founders know that by the cooling of a casting, it is specially on this spot that the defects of leakage are produced, by the formation of cracks and by obtaining cast-iron of porous constitution.

By the interposition of a metal sheet according to the invention the following advantages are specially obtained:—

(1) The cylinder properly so called is

poured as having only a wall of uniform thickness, whereby the pouring operation is assured to be particularly regular, that is to say, without swells, jerks and shocks.

(2) The inconveniences of the contraction, produced by cooling on the spots as 8, where the variation of section is a sudden one, are prevented by the fact that the over-thickness is divided into two parts by the metal sheet, in such a manner that the contraction on these spots is produced as if there were on said spots two distinct pieces of normal thickness.

#### Claims.

1. A casting having relatively thick and relatively thin portions, in combination with metal sheets, the sheets being positioned on the surfaces of the relatively thin portions, and embedded in the casting in the relatively thick portions, so as to be enveloped by the casting, the changes from the surface positioning to the embedded positioning occurring at points where there is an abrupt change of thickness in the casting.

2. A casting according to claim 1, the changes from said surface molding, to said envelopment by the cast metal, occurring at points where there is an abrupt change of thickness in the casting.

In testimony whereof I affix my signature in presence of two witnesses.

ERNEST MAYER.

Witnesses:

LEONARD LEVER,

GEORGES VANDER HAEGHEN.